

Sept. 16, 1958

J. E. JONES

2,852,385

SUPERSENSITIZATION OF PHOTOGRAPHIC EMULSIONS

Filed May 14, 1956

**Fig. 1**



A = 3,3'-DIETHYLOXATHIADICARBOCYANINE IODIDE  
B = 2-*p*-DIETHYLAMINOBENZALAMINOBENZOTHIAZOLE  
C = 3,3'-DIETHYLOXATHIADICARBOCYANINE IODIDE PLUS  
2-*p*-DIETHYLAMINOBENZALAMINOBENZOTHIAZOLE

**Fig. 2**



A = 3,3'-DIETHYLOXATHIADICARBOCYANINE IODIDE  
D = 2-*p*-DIETHYLAMINOSTYRYLBENZOTHIAZOLE  
E = 3,3'-DIETHYLOXATHIADICARBOCYANINE IODIDE PLUS  
2-*p*-DIETHYLAMINOSTYRYLBENZOTHIAZOLE

**Fig. 3**



A = 3,3'-DIETHYLOXATHIADICARBOCYANINE IODIDE  
F = 2-[4-(*p*-DIMETHYLAMINOPHENYL)-1,3-BUTADIENYL] BENZOTHIAZOLE  
G = 3,3'-DIETHYLOXATHIADICARBOCYANINE IODIDE PLUS 2-[4-(*p*-DIMETHYLAMINOPHENYL)-1,3-BUTADIENYL] BENZOTHIAZOLE

**Jean E. Jones**

INVENTOR.

*Daniel L. Mayne*  
BY  
*Lawrence H. Willis*  
ATTORNEY

# United States Patent Office

2,852,385

Patented Sept. 16, 1958

1

2,852,385

## SUPERSENSITIZATION OF PHOTOGRAPHIC EMULSIONS

Jean E. Jones, Rochester, N. Y., assignor to Eastman Kodak Company, Rochester, N. Y., a corporation of New Jersey

Application May 14, 1956, Serial No. 584,553

16 Claims. (Cl. 96—104)

This invention relates to photographic silver halide emulsions useful in color photography and photographic silver halide emulsions containing dicarbocyanine dyes, and as supersensitizers therefor, styryl-type bases.

It is known in the art of making photographic emulsions that certain dyes of the cyanine class alter the sensitivity of photographic emulsions of the gelatino-silver-halide kind, when the dyes are incorporated in the emulsions. It is also known that the sensitization produced by a given dye varies somewhat with the type of emulsion in which the dye is incorporated. Furthermore, the sensitization of a given emulsion by a given dye may be altered by varying the conditions in the emulsion. For example, the sensitization may be increased by increasing the silver ion concentration or decreasing the hydrogen ion concentration (i. e., increasing the alkalinity) or both. Thus, sensitization can be increased by bathing plates, coated with a spectrally sensitized emulsion, in water or in aqueous solutions of ammonia. Such a process of altering the sensitivity of a sensitized emulsion by increasing the silver ion concentration and/or by decreasing the hydrogen ion concentration is commonly called "hypersensitization." Hypersensitized emulsions have generally poor keeping qualities.

I have now found another means of altering the sensitivity in emulsions containing dicarbocyanine dyes. Since the conditions in the emulsion, i. e., the hydrogen ion and/or the silver ion concentration undergo little or no change in my method, I shall designate my method as a kind of supersensitization.

It is, therefore, an object of my invention to provide photographic emulsions containing dicarbocyanine dyes and, as supersensitizers therefor, styryl-type bases. Another object is to provide a process for preparing these supersensitized emulsions. Other objects will become apparent from a consideration of the following description and examples.

The dicarbocyanine dyes which are useful in practicing my invention include those represented by the following general formula:



wherein R and R<sub>1</sub> each represents an alkyl group (such as methyl, ethyl,  $\beta$ -hydroxyethyl, carboxymethyl,  $\beta$ -carboxyethyl, carbomethoxymethyl, carbethoxymethyl, etc., n represents a positive integer of from 1 to 2, X represents an acid radical, such as chloride, iodide, bromide, perchlorate, p-toluenesulfonate, benzenesulfonate, ethylsulfate, methylsulfate, etc., Z represents the non-metallic atoms necessary to complete a heterocyclic nucleus containing from 5 to 6 atoms in the heterocyclic ring, e. g., a heterocyclic nucleus of the benzothiazole series (e. g., benzothiazole, 4-chlorobenzothiazole, 5-chlorobenzothiazole, 6-chlorobenzothiazole, 7-chlorobenzothiazole, 4-methylbenzothiazole, 5-methylbenzothiazole, 6-methylbenzothiazole, 5-bromobenzothiazole, 6-bromobenzothiazole, 6-methyl-5-bromobenzothiazole, etc.)

2

zole, 4-phenylbenzothiazole, 5-phenylbenzothiazole, 4-methoxybenzothiazole, 5-methoxybenzothiazole, 6-methoxybenzothiazole, 6-iodobenzothiazole, 5-iodobenzothiazole, 4-ethoxybenzothiazole, 5-ethoxybenzothiazole, 5,6-dimethylbenzothiazole, 5-hydroxybenzothiazole, 6-hydroxybenzothiazole, etc.) a heterocyclic nucleus of the naphthothiazole series (e. g.,  $\alpha$ -naphthothiazole,  $\beta$ -naphthothiazole, 7-methoxy- $\alpha$ -naphthothiazole, 8-methoxy- $\alpha$ -naphthothiazole, 5-methoxy- $\beta$ -naphthothiazole, 5-ethoxy- $\alpha$ -naphthothiazole, etc.), a heterocyclic nucleus of the benzoselenazole series (e. g., benzoselenazole, 5-chlorobenzoselenazole, 6-methoxybenzoselenazole, 5-methoxybenzoselenazole, etc.), a heterocyclic nucleus of the naphthoselenazole series (e. g.,  $\alpha$ -naphthoselenazole,  $\beta$ -naphthoselenazole, etc.), a heterocyclic nucleus of the benzoxazole series (e. g., benzoxazole, 5-hydroxybenzoxazole, 6-hydroxybenzoxazole, 5-chlorobenzoxazole, 5-methoxybenzoxazole, 6-methoxybenzoxazole, 5-phenylbenzoxazole, 5-bromobenzoxazole, etc.), a heterocyclic nucleus of the naphthoxazole series (e. g.,  $\alpha$ -naphthoxazole,  $\beta$ -naphthoxazole, etc.), a heterocyclic nucleus of the 2-quinoline series (e. g., 2-quinoline, 6-methyl-2-quinoline, 7-methyl-2-quinoline, 8-methyl-2-quinoline, 6-chloro-2-quinoline, 8-chloro-2-quinoline, 4-chloro-2-quinoline, 5-ethoxy-2-quinoline, 6-ethoxy-2-quinoline, 7-ethoxy-2-quinoline, 6-hydroxy-2-quinoline, 7-hydroxy-2-quinoline, 6-methoxy-2-quinoline, etc.), a heterocyclic nucleus of the 4-quinoline series (e. g., 4-quinoline, 6-methoxy-4-quinoline, 7-methyl-4-quinoline, 8-methyl-4-quinoline, etc.), a heterocyclic nucleus of the benzimidazole series (e. g., benzimidazole, 5-chlorobenzimidazole, 5,6-dichlorobenzimidazole, 1,7-trimethylenebenzimidazole, etc.), a heterocyclic nucleus of the 5,6-benzoquinoline series (e. g., 5,6-benzo-2-quinoline, etc.), etc., and Z<sub>1</sub> represents the non-metallic atoms necessary to complete a heterocyclic nucleus selected from the group consisting of those of the benzoxazole series (e. g., such as those defined by Z above), those of the naphthoxazole series (e. g., such as those defined by Z above), those of the benzoselenazole series (e. g., such as those defined by Z above), those defined by Z above), those of the naphthoselenazole series (e. g., such as those defined by Z above), those of the benzothiazole series (e. g., such as those defined by Z above), those of the naphthothiazole series (e. g., such as those defined by Z above), etc. Other carbocyanine dyes can also be employed in my invention.

45 The styryl-type bases useful in practicing my invention can advantageously be represented by the following general formulas:

II.



and

III.



55 wherein R<sub>2</sub> represents a monocyclic aryl group of the benzene series, such as phenyl, dimethylaminophenyl (o-, m-, or p-), diethylaminophenyl (o-, m-, or p-), aminophenyl (o-, m-, or p-), hydroxyphenyl (o-, m-, or p-), chlorophenyl (o-, m-, or p-), etc., n represents a positive integer of from 1 to 2, L represents a nitrogen atom or a methine group, i. e.,  $-\text{CR}_3-$  wherein R<sub>3</sub> is a hydrogen atom, a cyano group, an alkoxyl group (methoxyl, ethoxyl, etc., for example), etc., and Z<sub>2</sub> represents the non-metallic atoms necessary to complete a heterocyclic nucleus, such as those of the thiazole series, those of the benzothiazole series, those of the naphthothiazole series, those of the oxazole series, those of the benzoxazole series, those of the naphthoxazole series, those of the selenazole series, those of the benzoselenazole series, those of the naphthoselenazole series, those of the perinaphtho-1,3-thiazine series, those of the 2-quinoline series (n is 1),

those of the 4-quinoline series (*n* is 2); those of the 2-pyridine series (*n* is 1), those of the benzimidazole series, etc. The hydrogen atoms of these heterocyclic nuclei can be substituted by the usual groups which have no adverse effects on the emulsions, such as chlorine, bromine, methyl, ethyl, phenyl, hydroxyl, methoxyl, ethoxyl, etc. These styryl-type bases can be prepared by methods well known to those skilled in the art. For example, these styryl-type bases can be prepared by condensing a heterocyclic base containing a reactive amino or methyl group with an aromatic aldehyde. Alternatively, they can be prepared by dequaternization of the corresponding styryl dyes, as described in U. S. Patent 2,169,434, issued August 15, 1939. Listed below are representative styryl-type bases of Formulas II or III which can advantageously be employed in my invention.



According to my invention, I incorporate one or more of the dicarbocyanine dyes represented by Formula I above with one or more styryl-type bases, such as those represented by Formulas II or III above. My invention is particularly directed to the ordinarily employed gelatino-silver-halide emulsions. However, my supersensitizing combinations can be employed in silver halide emulsions in which the carrier is other than gelatin, e. g., a resinous substance or cellulosic material which has no deteriorating effect on the light-sensitive materials. The dicarbocyanine dyes and styryl-type bases can be employed in various concentrations depending upon the effects desired.

Ordinarily, the optimum or near optimum concentration of the dicarbocyanine dyes which I employ in practicing my invention is of the order of from 0.010 to 0.30 g. per mol. of silver halide in the emulsion.

The styryl-type bases which I employ in my invention can advantageously be employed at a concentration of

from about 0.010 to 1.0 g. per mol. of silver halide in the emulsion.

In general, the ratio of concentration of dicarbocyanine dye to styryl-type base can vary rather widely in my combination, e. g. from 1:1 to 1:100 (by weight) in many cases.

The methods of incorporating sensitizing dyes and styryl-type bases in silver halide emulsions are well known to those skilled in the art. While the dicarbocyanine dyes and styryl-type bases can be directly dispersed in the emulsions, it is convenient to add the same in the form of solutions in appropriate solvents. Methanol, ethanol, pyridine, and the like have proven satisfactory for many of the dyes of Formula I and bases of Formulas II and III. Mixtures of solvents, e. g., pyridine diluted with methanol or acetone, can also be used. The dicarbocyanine dyes and styryl-type bases are dispersed in the finished emulsions and should be uniformly distributed throughout the emulsions. The following procedure is

resented by Formula I above, and (2) a combination of the dicarbocyanine dye and styryl-type base. Then the emulsions were held at about 50-52° C. for a short time and coated on a support, chill set, and dried. After exposure through a Wratten No. 25 filter, i. e., a filter which transmits substantially no light of wavelength shorter than about 580 mu, in an Eastman Type Ib sensitometer, the film strips were processed for 3 minutes in a developer having the following composition:

|    |                                |       |      |
|----|--------------------------------|-------|------|
| 10 | N-methyl-p-aminophenol sulfate | g     | 2.0  |
|    | Hydroquinone                   | g     | 8.0  |
|    | Sodium sulfite (desiccated)    | g     | 90.0 |
|    | Sodium carbonate (monohydrate) | g     | 52.5 |
| 15 | Potassium bromide              | g     | 5.0  |
|    | Water to make                  | liter | 1    |

The speed (red), gamma and fog for each of the coatings was then measured. The results are recorded in Table I.

TABLE I

| Example | Sensitizing Dye and Base (g./mol. AgX)                              | Red Light Exposure |       |     |
|---------|---------------------------------------------------------------------|--------------------|-------|-----|
|         |                                                                     | 30/E<br>Speed      | Gamma | Fog |
| 1.      | {(a) 3,3'-diethyloxathiadcarbocyanine iodide (.045)-                | 4.05               | 1.30  | .06 |
|         | {(b) dye (a) (.045) with base 1 (.15)-                              | 17.7               | 2.70  | .08 |
| 2.      | {(c) dye (a) (.045)-                                                | 4.15               | 1.39  | .08 |
|         | {(d) dye (a) (.045) with base 2 (.15)-                              | 35.0               | 1.69  | .08 |
| 3.      | {(e) dye (a) (.045) with base 3 (.15)-                              | 18.0               | 1.60  | .08 |
| 4.      | {(f) dye (a) (.045) with base 4 (.15)-                              | 19.0               | 1.55  | .06 |
| 5.      | {(g) dye (a) (.045) with base 5 (.15)-                              | 13.1               | 1.55  | .06 |
| 6.      | {(h) dye (a) (.045) with base 6 (.15)-                              | 15.8               | 1.69  | .06 |
| 7.      | {(i) dye (a) (.045)-                                                | 3.45               | 1.14  | .05 |
|         | {(j) dye (a) (.045) with base 7 (.15)-                              | 9.05               | 2.10  | .08 |
| 8.      | {(k) 3,3'-diethylthiadcarbocyanine iodide (.045)-                   | 5.1                | 1.1   | .05 |
|         | {(l) dye (k) (.045) with base 2 (.15)-                              | 28.0               | 1.8   | .06 |
| 9.      | {(m) 3,3'-diethylselenadcarbocyanine iodide (.045)-                 | 4.2                | 1.2   | .06 |
|         | {(n) dye (m) (.045) with base 2 (.15)-                              | 16.9               | 2.0   | .05 |
| 10.     | {(o) 3,3'-diethyl-4,5,4',5'-dibenzothiadcarbocyanine iodide (.045)- | 2.4                | 1.0   | .07 |
|         | {(p) dye (o) (.045) with base 2 (.15)-                              | 8.5                | 2.0   | .07 |
| 11.     | {(q) 3,3'-diethyloxadiacarbocyanine bromide (.045)-                 | 3.6                | 1.8   | .07 |
|         | {(r) dye (q) (.045) with base 2 (.15)-                              | 45.5               | 2.4   | .08 |
| 12.     | {(s) dye (a) (.050)-                                                | 2.0                | .50   | .05 |
|         | {(t) dye (a) (.050) with base 8 (.08)-                              | 15.0               | 1.5   | .05 |
| 13.     | {(u) dye (a) (.050) with base 9 (.08)-                              | 5.4                | 1.3   | .05 |
| 14.     | {(v) dye (a) (.050) with base 10 (.08)-                             | 3.8                | 1.0   | .08 |
| 15.     | {(w) dye (a) (.050) with base 11 (.08)-                             | 3.0                | .78   | .06 |
| 16.     | {(x) dye (a) (.050) with base 12 (.08)-                             | 10.6               | 1.8   | .05 |
| 17.     | {(y) dye (a) (.050) with base 13 (.08)-                             | 7.1                | 1.4   | .06 |
| 18.     | {(z) dye (a) (.050) with base 14 (.08)-                             | 5.4                | .60   | .05 |
| 19.     | {(a') dye (a) (.050) with base 15 (.08)-                            | 15.8               | 1.7   | .06 |
| 20.     | {(b') dye (a) (.050) with base 16 (.08)-                            | 17.7               | 1.8   | .08 |
| 21.     | {(c') dye (a) (.050) with base 17 (.08)-                            | 28.5               | 1.9   | .05 |

satisfactory: Stock solutions of the dicarbocyanine dyes and styryl-type bases are prepared by dissolving the same in appropriate solvents as described above. Then, to the flowable gelatino-silver-halide emulsion, the desired amounts of the stock solution of one of the dyes (or styryl-type bases) are slowly added, while stirring the emulsion. Stirring is continued until the dye is thoroughly incorporated in the emulsion. Then the desired amount of the stock solution of the styryl-type base (or dye, if styryl-type base has been added first) is slowly added to the emulsion, while stirring. Stirring is continued until the second solution is thoroughly incorporated. The supersensitized emulsion can then be coated out on a suitable support, such as glass, cellulose derivative film, resin film, or paper, to a suitable thickness and allowed to dry. The details of such coating methods are well known to those skilled in the art. The foregoing procedures and proportions are to be regarded only as illustrative. Clearly, my invention is directed to any silver halide emulsion containing a combination of the aforesaid dicarbocyanine dyes and styryl-type bases whereby a supersensitizing effect is obtained.

The following examples will serve to illustrate further the manner of practicing my invention.

In Table I below, to different portions of the same batch of photographic gelatino-silver-bromide emulsion were added (1) a dicarbocyanine dye, such as those rep-

50 5 and 6 were made from the same batch of emulsion and the coatings of Examples 12 to 21 were made from the same batch of emulsion. No measurements of coatings containing only the styryl-type bases alone are given, since numerous coatings at the concentrations used in 55 the table have shown that these bases alone have little or no measurable sensitizing effect on the emulsions.

My invention is primarily directed to the ordinarily employed gelatino-silver-halide developing-out emulsions, e. g., gelatino-silver-chloride, -chlorobromide, -chlorooiodide, -chlorobromide, -bromide and -bromiodide developing-out emulsions. Emulsions which form the latent image mostly inside the silver halide grains, such as the emulsions set forth in U. S. Patent 2,456,956, dated December 21, 1948, can also be employed in practicing my 65 invention.

The emulsions prepared in accordance with my invention can be coated in the usual manner on any suitable support, e. g., glass, cellulose nitrate film, cellulose acetate film, polyvinylacetal resin film, paper or metal.

70 Photographic silver halide emulsions, such as those listed above, containing the supersensitizing combinations of my invention can also contain such addenda as chemical sensitizers, e. g., sulfur sensitizers (e. g., allyl thiocarbamide, thiourea, allylisothiocyanate, cystine, etc.), various gold compounds (e. g., potassium chloroaurate,

auric trichloride, etc.) (See U. S. Patents 2,540,085; 2,597,856 and 2,597,915), various palladium compounds, such as palladium chloride (U. S. 2,540,086), potassium chloropalladate (U. S. 2,598,079), etc., or mixtures of such sensitizers; antifoggants, such as ammonium chloroplatinate (U. S. 2,566,245), ammonium chloroplatinite (U. S. 2,566,263), benzotriazole, nitrobenzimidazole, 5-nitroindazole, benzidine, mercaptans, etc. (see Mees—"The Theory of the Photographic Process," Macmillan Pub., 1942, page 460), or mixtures thereof; hardeners, such as formaldehyde (U. S. 1,763,533), chrome alum (U. S. 1,763,533), glyoxal (U. S. 1,870,354), dibromacrolein (Br. 406,750), etc.; color couplers, such as those described in U. S. Patent 2,423,730, Spence and Carroll U. S. Patent 2,640,776, etc.; or mixtures of such addenda. Dispersing agents for color couplers, such as those set forth in U. S. Patents 2,322,027 and 2,304,940, can also be employed in the above-described emulsions.

As noted above, methods for preparing the styryl-type bases of my invention represented by Formulas II and III above have been previously described in the prior art. The following example will illustrate the preparation of the compounds of Formula II wherein L represents a nitrogen atom.

*Example A.—2-p-diethylaminobenzalaminobenzothiazole*



An intimate mixture of 1.5 g. (1. mol.) of 2-aminobenzothiazole and 1.8 g. (1. mol.) of p-diethylaminobenzaldehyde was heated, with stirring, in a test tube over a free flame for three minutes. The deep orange sticky mass was dissolved in 2 ml. of methyl alcohol, the solution was stirred with 10 ml. of ether and the whole chilled for one hour in a freezing mixture of ice and acetone. The crystals were collected on a filter and washed with ether. The yield of dye was 15% crude, 8% after four recrystallizations from ligroin (B. P. 66-75° C.) and 3% after a further recrystallization from aqueous alcohol. The orange crystals melted at 95-96° C. with decomposition.

Listed below are a number of compounds, together with literature references describing the preparation thereof.

| Styryl-type Base | Reference                             |
|------------------|---------------------------------------|
| 9.....           | Bellstein, vol. 20, page 497.         |
| 10.....          | Chemical Abstracts, vol. 32, pg. 169. |
| 14.....          | Bellstein, vol. 21, page 149.         |
| 15.....          | Jour. Chem. Soc., 1943, page 491.     |
| 16.....          | Bellstein, vol. 27, page 385.         |
| 17.....          | Chemical Abstracts, vol. 31, pg. 400. |

Listed below are melting points for a number of the styryl-type bases of my invention which were prepared exactly according to the methods described in the above prior art references.

| Styryl-type Base | Melting Point                      |
|------------------|------------------------------------|
| 3.....           | 130-132° C. with dec.              |
| 5.....           | 113-114° C.                        |
| 7.....           | 188-190° C.                        |
| 8.....           | 142-143° C.                        |
| 13.....          | 60-62° C. with previous shrinking. |

The preparation of a number of styryl-type base compounds which can be used in my invention is described in Brooker and Sprague U. S. Patent 2,345,094, issued March 28, 1944. A number of the styryl dyes which can be dequaternated to produce bases useful in practicing my invention have been described in Brooker and White U. S. Patent 2,494,032, issued January 10, 1950.

While it has been noted that certain styryl dyes can be employed in supersensitizing combinations with the

dicarbocyanine dyes of my invention, these styryl dyes do not generally provide the consistent results illustrated in the above examples with respect to the styryl-type bases. It has been found, for example, that the styryl dye, 2-p-dimethylaminostyrylbenzoxazole ethiodide, can be employed in supersensitizing combination with various dicarbocyanine dyes, such as dye a of Table I.

The accompanying drawing illustrates the supersensitizing effect obtained with three of my new combinations of dyes in gelatino-silver-bromide emulsions. Each figure in the drawing is a diagrammatic reproduction of three spectrograms. In each figure, the sensitivity of the emulsion containing only the dicarbocyanine dye of Formula I is represented by the solid curve, the sensitivity of the same emulsion containing only the styryl-type base of Formula II or III is represented by the curve consisting of dotted lines, while the sensitivity of the same emulsion containing both the dicarbocyanine dye of Formula I and the styryl-type base of Formula II or III is represented by the curve consisting of alternating long and short lines. It will be noted that the maximum sensitizing action for the styryl-type bases generally occurs in the green light region of the spectrum, hence, emulsions containing these styryl-type bases generally show little or no speed to red light, as can be seen by reference to Table I above.

In Fig. 1, curve A represents the sensitivity of an ordinary gelatino-silver-bromide emulsion sensitized with 3,3'-diethyloxathiadicarbocyanine iodide, curve B represents the sensitivity of the same emulsion sensitized with 2-p-diethylaminobenzalaminobenzothiazole, while curve C represents the sensitivity of the same emulsion sensitized with both 3,3'-diethyloxathiadicarbocyanine iodide and 2-p-diethylaminobenzalaminobenzothiazole.

In Fig. 2, curve A represents the sensitivity of an ordinary gelatino-silver-bromide emulsion sensitized with 3,3'-diethyloxathiadicarbocyanine iodide, curve D represents the sensitivity of the same emulsion sensitized with 2-p-diethylaminostyrylbenzothiazole, while curve E represents the sensitivity of the same emulsion sensitized with both 3,3'-diethyloxathiadicarbocyanine iodide and 2-p-diethylaminostyrylbenzothiazole. Sensitometric measurements for emulsions sensitized in the manner shown in Fig. 2 are given in Example 8 of the above table.

In Fig. 3, curve a represents the sensitivity of an ordinary gelatino-silver-bromide emulsion sensitized with 3,3'-diethyloxathiadicarbocyanine iodide, curve F represents the sensitivity of the same emulsion sensitized with 2-[4-(p-dimethylaminophenyl)-1,3-butadienyl] benzothiazole, while curve G represents the sensitivity of the same emulsion sensitized with 3,3'-diethyloxathiadicarbocyanine iodide and 2-[4-(p-dimethylaminophenyl)-1,3-butadienyl] benzothiazole.

What I claim as my invention and desire secured by Letters Patent of the United States is:

1. A photographic silver halide emulsion sensitized with a supersensitizing combination of at least one dicarbocyanine dye selected from those represented by the following general formula:



wherein R and R<sub>1</sub> each represents an alkyl group, n represents a positive integer of from 1 to 2, X represents an acid radical, Z represents the non-metallic atoms necessary to complete a heterocyclic nucleus selected from the group consisting of those of the benzothiazole series, those of the naphthothiazole series, those of the benzoselenazole series, those of the benzoxazole series, those of the naphthoxazole series, those of the 2-quinoline series, those of the 4-quinoline series, and those of the benzimidazole series, and Z<sub>1</sub> represents the non-metallic atoms necessary to complete a heterocyclic nucleus selected

from the group consisting of those of the benzoxazole series, those of the naphthoxazole, those of the benzoselenazole series, those of the naphthoselenazole series, those of the benzothiazole series, and those of the naphthothiazole series, and at least one heterocyclic base selected from the group consisting of those represented by the following two general formulas:



and



wherein  $Z_2$  represents the non-metallic atoms necessary to complete a heterocyclic nucleus selected from the group consisting of those of the thiazole series, those of the benzothiazole series, those of the naphthothiazole series, those of the benzoxazole series, those of the benzoselenazole series, those of the perinaphtho-1,3-thiazine series, those of the benzimidazole series, those of the 2-quinoline series, those of the 4-quinoline series, and those of the 2-pyridine series, L represents a member selected from the group consisting of a nitrogen atom and a methine group,  $R_2$  represents an aryl group, and  $n$  represents a positive integer of from 1 to 2.

2. A photographic gelatino-silver-halide developing-out emulsion sensitized with a supersensitizing combination of methine group.  $R_2$  represents an aryl group, and  $n$  represented by the following general formula:



wherein R and  $R_1$  each represents an alkyl group containing from 1 to 2 carbon atoms,  $n$  represents a positive integer of from 1 to 2, X represents an acid radical, Z represents the non-metallic atoms necessary to complete a heterocyclic nucleus selected from the group consisting of those of the benzothiazole series, those of the naphthothiazole series, those of the benzoxazole series, those of the naphthoxazole series, those of the 2-quinoline series, those of the 4-quinoline series, and those of the benzimidazole series, and  $Z_1$  represents the nonmetallic atoms necessary to complete a heterocyclic nucleus selected from the group consisting of those of the benzoxazole series, those of the naphthoxazole series, those of the benzoselenazole series, those of the benzothiazole series, those of the naphthoselenazole series, those of the benzothiazole series, and those of the naphthothiazole series, and at least one heterocyclic base selected from the group consisting of those represented by the following two general formulas:



and



wherein  $Z_2$  represents the non-metallic atoms necessary to complete a heterocyclic nucleus selected from the group consisting of those of the thiazole series, those of the benzothiazole series, those of the naphthothiazole series, those of the benzoxazole series, those of the benzoselenazole series, those of the perinaphtho-1,3-thiazine series, those of the benzimidazole series, those of the 2-quinoline series, those of the 4-quinoline series, and those of the 2-pyridine series, L represents a member selected from the group consisting of a nitrogen atom and a methine group,  $R_2$  represents a monocyclic aryl group of the benzene series, and  $n$  represents a positive integer of from 1 to 2.

3. A photographic gelatino-silver-halide developing-

out emulsion sensitized with a supersensitizing combination of at least one dicarbocyanine dye selected from those represented by the following general formula:



wherein R and  $R_1$  each represents an alkyl group containing from 1 to 2 carbon atoms,  $n$  represents a positive integer of from 1 to 2, X represents an acid radical, Z represents the non-metallic atoms necessary to complete a heterocyclic nucleus selected from the group consisting of those of the benzothiazole series, those of the naphthothiazole series, those of the benzoxazole series, those of the benzoselenazole series, those of the naphthoxazole series, those of the 2-quinoline series, those of the 4-quinoline series, and those of the benzimidazole series, and  $Z_1$  represents the non-metallic atoms necessary to complete a heterocyclic nucleus selected from the group consisting of those of the benzoxazole series, those of the naphthoxazole series, those of the benzoselenazole series, those of the benzothiazole series, those of the naphthoselenazole series, those of the benzothiazole series, and those of the naphthothiazole series, and at least one heterocyclic base selected from those represented by the following general formula:



wherein  $Z_2$  represents the non-metallic atoms necessary to complete a heterocyclic nucleus selected from the group consisting of those of the thiazole series, those of the benzothiazole series, those of the naphthothiazole series, those of the benzoxazole series, those of the benzoselenazole series, those of the perinaphtho-1,3-thiazine series, those of the benzimidazole series, those of the 2-quinoline series, those of the 4-quinoline series, and those of the 2-pyridine series, L represents a member selected from the group consisting of a nitrogen atom and a methine group,  $R_2$  represents a monocyclic aryl group of the benzene series, and  $n$  represents a positive integer of from 1 to 2.

4. A photographic gelatino-silver-halide developing-out emulsion sensitized with a supersensitizing combination of at least one dicarbocyanine dye selected from those represented by the following general formula:



wherein R and  $R_1$  each represents an alkyl group containing from 1 to 2 carbon atoms, X represents an acid radical, Z represents the non-metallic atoms necessary to complete a heterocyclic nucleus of the benzothiazole series and  $Z_1$  represents the non-metallic atoms necessary to complete a heterocyclic nucleus of the benzoxazole series, and at least one heterocyclic base selected from those represented by the following general formula:



wherein  $Z_2$  represents the non-metallic atoms necessary to complete a heterocyclic nucleus selected from the group consisting of those of the thiazole series, those of the benzothiazole series, those of the naphthothiazole series, those of the benzoxazole series, those of the benzoselenazole series, those of the perinaphtho-1,3-thiazine series, those of the benzimidazole series, those of the 2-quinoline series, and those of the 2-pyridine series, L represents a member selected from the group consisting of a nitrogen atom and a methine group, and  $R_2$  represents a monocyclic aryl group of the benzene series.

5. A photographic gelatino-silver-halide developing-out emulsion sensitized with a supersensitizing combination of



wherein  $Z_2$  represents the non-metallic atoms necessary to complete a heterocyclic nucleus of the naphthothiazole series, and  $R_2$  represents a monocyclic aryl group of the benzene series.

14. A photographic gelatino-silver-halide developing-out emulsion sensitized with a supersensitizing combination of 3,3'-diethyloxathiadicarbocyanine iodide and 2-p-dimethylaminostyryl- $\alpha$ -naphthothiazole.

15. A photographic gelatino-silver-halide developing-out emulsion sensitized with a supersensitizing combination of at least one dicarbocyanine dye selected from those represented by the following general formula:



5

and at least one heterocyclic base selected from those represented by the following general formula:



10

wherein  $Z_2$  represents the non-metallic atoms necessary to complete a heterocyclic nucleus of the benzimidazole series, and  $R_2$  represents a monocyclic aryl group of the benzene series.

16. A photographic gelatino-silver-halide developing-out emulsion sensitized with a supersensitizing combination of 3,3'-diethyloxathiadicarbocyanine iodide and 2-styrylbenzimidazole.

#### References Cited in the file of this patent

#### UNITED STATES PATENTS

|           |                    |       |               |
|-----------|--------------------|-------|---------------|
| 2,075,046 | Mees               | ----- | Mar. 30, 1937 |
| 2,313,922 | Carroll et al.     | ----- | Mar. 16, 1943 |
| 2,448,858 | Carroll et al.     | ----- | Sept. 7, 1948 |
| 2,680,686 | Van Dormael et al. | ----- | June 8, 1954  |

#### FOREIGN PATENTS

|         |           |       |              |
|---------|-----------|-------|--------------|
| 110,697 | Australia | ----- | May 24, 1940 |
|---------|-----------|-------|--------------|

UNITED STATES PATENT OFFICE  
CERTIFICATE OF CORRECTION

Patent No. 2,852,385

Jean E. Jones

September 16, 1958

It is hereby certified that error appears in the printed specification of the above numbered patent requiring correction and that the said Letters Patent should read as corrected below.

Column 2, line 32, for "trimethylenebenizimidazole" read -- trimethylenebenzimidazole --; column 8, line 45, for "In Fig. 3, curve a" read -- In Fig. 3, curve A --; column 9, line 29, for "methine group. R<sub>2</sub> represents an aryl group, and n" read -- at least one dicarbocyanine dye selected from those --; column 12, line 26, for "seires" read -- series --.

Signed and sealed this 30th day of December 1958.

(SEAL)  
Attest:

KARL H. AXLINE

Attesting Officer

ROBERT C. WATSON  
Commissioner of Patents